

# United States Patent

Anderson

[15] 3,652,330

[45] Mar. 28, 1972

[54] **PROCESS FOR COATING AMORPHOUS SELENIUM**

[72] Inventor: Donald E. Anderson, Northfield, Minn.

[73] Assignee: G. T. Schjeldahl Company, Northfield, Minn.

[22] Filed: Sept. 14, 1970

[21] Appl. No.: 71,671

[52] U.S. Cl.....117/201, 117/101, 117/107

[51] Int. Cl.....G03g 7/00

[58] Field of Search.....117/200, 201, 106, 107, 101

[56] **References Cited**

UNITED STATES PATENTS

3,019,129 1/1962 Walsh.....117/101

Primary Examiner—William L. Jarvis

Attorney—Orrin M. Haugen

[57]

## ABSTRACT

The method of applying a film of amorphous selenium to a substrate having a generally cylindrical surface, the method comprising inserting a charge of selenium into a generally cylindrical crucible having an inner wall extending in spaced relationship to a cylindrical axis, and treating the selenium charged therein so as to dispose the charge generally along the walls of the crucible so as to define a generally cylindrical charge profile uniformly spaced about the crucible axis. This treatment is preferably accomplished by the rotation of the crucible about its axis at a rate sufficient to centrifugally force the charge to a uniformly cylindrically profiled form. The charge is thereafter heated to a temperature at least sufficient to cause sublimation of the selenium within the crucible, while the charge is rotated about its axis at a rate sufficient to hold the charge uniformly about the inner crucible wall. While this is occurring, the substrate is inserted into the crucible with the outer cylindrical surface being spaced a predetermined distance from the surface of the cylindrical charge profile. During the deposition of the selenium onto the substrate surface, the substrate is chilled to a temperature ranging from between about 50° C. and 70° C.

5 Claims, 10 Drawing Figures



PATENTED MAR 28 1972

3,652,330

SHEET 1 OF 3



FIG 1



## FIG 2

INVENTOR.  
DONALD E. ANDERSON  
*Darin M. Haugen*  
ATTORNEY

PATENTED MAR 28 1972

3,652,330

SHEET 2 OF 3



FIG 3



**FIG 4**

INVENTOR  
DONALD E. ANDERSON  
BY *Orvin M. Haugen*  
ATTORNEY

PATENTED MAR 28 1972

3,652,330

SHEET 3 OF 3



**FIG 6**



**FIG 7a**



**FIG 9**



**FIG 7b**



**FIG 8**

INVENTOR.  
DONALD E. ANDERSON  
BY  
*Dorin M. Daugler*  
ATTORNEY

## PROCESS FOR COATING AMORPHOUS SELENIUM

## CROSS-REFERENCE TO RELATED APPLICATIONS

The present invention relates to a method for the deposition of amorphous selenium on substrate surfaces, the process being conducted in that certain coating apparatus described in my co-pending application Ser. No. 20,643, filed Mar. 18, 1970, entitled "Method and Apparatus for Coating Articles Utilizing Rotating Crucible," and assigned to the same assignee as the present invention.

## BACKGROUND OF THE INVENTION

The present invention relates generally to an improved technique for applying a film of amorphous selenium to a substrate surface, and more specifically to an improved technique for the preparation of amorphous selenium films which have properties desirable for reprographic applications, and in particular, xerographic applications. The process of the present invention provides for the preparation of the rapid, uniform and isothermal deposition of a film of selenium on the surface of a substrate member, the selenium having unusual and desirable properties for use in the reprographics area.

In the past, evaporative or sublimation deposition techniques have been utilized for the preparation of selenium coatings, the systems normally including a stationary crucible and a movable substrate. These techniques, which are time-consuming and difficult to control, are normally wasteful of selenium, and provide finished films which tend toward incipient crystallization, and which possess a tendency toward "onionskinning" or layering.

In accordance with the process of the present invention, however, a selenium retaining crucible is provided which is preferably in the form of a right circular cylinder, the crucible being heated from an externally disposed source, and being arranged to be rotated about its central axis. The rate of rotation is sufficient to provide for sufficient centrifugal force so as to eliminate the danger of splattering of evaporant under the evaporating or subliming conditions. The substrate being coated is mounted on a suitable collet or other device for insertion into the rotating crucible, and for retention therein during the coating operation. Thermal control means are provided which cooperate with the collet for maintaining surface contact with the substrate being coated, the contact being along a surface which is preferably concealed from the evaporant. Upon completion of the selenium coating operation, the article is removed from the chamber. If desired, baffle or shutter means may be utilized to prevent selenium deposition from occurring during the insertion and extraction operations. Also, suitably tapered baffle means may be utilized to accommodate a specifically programmed substrate insertion and extraction operation.

In the preparation of selenium films of uniform thickness along the Z axis, large source-to-substrate spacings are normally required. The method of the present invention eliminates the requirement of large spacing, and high production rates and reproducible devices having an amorphous structure may be fabricated. In this connection, deposition occurs substantially continuously and uniformly on the entire surface of the substrate, and not merely upon certain preselected surface areas, thereby affording better control of the entire system. It will be appreciated that the deposition occurs "continuously" and without interruption on each integral area of the substrate surface, and accordingly the entire substrate surface is exposed to a continuous application of selenium from the charge source either by the evaporation of the selenium or the sublimation of the selenium. Also, the process of the present invention simplifies temperature monitoring and temperature control of the substrate.

The rotating crucible provides a high degree of temperature "leveling" of the selenium source, and thus the resultant film is highly uniform, homogeneous, and amorphous. By controlling the distance between the surface of the selenium source and the surface of the substrate to a distance which is

less than the mean free path of the selenium evaporant within the system, relatively large changes in selenium reserve may be provided for in the crucible so as to accommodate sequential deposition onto many substrates.

5 The technique of the present invention is adaptable to both evaporative operations, and sublimation operations. Selenium films which are amorphous in their structure may be formed by either technique. In other words, it is not necessary that the temperature of the selenium charge be raised or elevated to 10 the melting point under the evaporative conditions. Therefore, when reference is made to "evaporative" operations, it will be understood that this also includes sublimation techniques as well.

15 Therefore, it is a primary object of the present invention to provide for an improved system for the preparation of evaporatively deposited amorphous selenium films, wherein the selenium films may be rapidly, uniformly, and isothermally deposited at high production rates, and in a reproducible fashion.

20 It is yet a further object of the present invention to provide an improved system for the preparation of evaporatively deposited amorphous selenium films, these films having unusual properties which render the products desirable for reprographic applications.

25 It is yet a further object of the present invention to provide an improved system for the preparation of amorphous selenium films, wherein a rotating crucible is employed in combination with a substrate retaining member which is non-rotating 30 and which is provided with means for closely controlling the temperature of the substrate.

35 Other and further objects of the present invention will become apparent to those skilled in the art upon a study of the following specification, appended claims and accompanying drawings.

## BRIEF DESCRIPTION OF THE DRAWINGS

FIG. 1 is a perspective view of a typical installation system for carrying out the selenium deposition of the present invention;

40 FIG. 2 is a detail perspective view of the substrate retaining collet, a substrate retaining magazine, and the rotating crucible apparatus illustrated in FIG. 1;

45 FIG. 3 is a sectional view of the selenium deposition system for carrying out the present invention, and illustrating the crucible oven, rotating crucible, and support collet useful in the systems shown in FIGS. 1 and 2;

50 FIG. 4 is a detail sectional view similar to FIG. 3, and illustrating the structure with shutter blades or baffles utilized in combination with the rotating crucible and source;

55 FIG. 5 is a vertical sectional view taken along the line and in the direction of the arrows 5-5 of FIG. 4;

55 FIG. 6 is a detail section view showing a preferred configuration or profile for the individual shutter blades;

FIGS. 7A and 7B illustrate the uncorrected and corrected deposition profile which is achieved through the utilization of a blade configuration such as is shown in FIG. 6;

60 FIG. 8 is a vertical sectional view taken along the longitudinal axis of the shutter blades shown in FIGS. 4, 5 and 6; and

65 FIG. 9 is a perspective view, partially in section, showing a cylindrical substrate having a coating of selenium thereon.

## DESCRIPTION OF THE PREFERRED EMBODIMENT

65 In order to describe the manner in which the process of the present invention may be carried out, particular attention is directed to FIG. 1 of the drawings which illustrates a typical installation which may be utilized for conducting the process 70 of the present invention. With reference to FIG. 1, it will be seen that the selenium deposition system generally designated 10 includes a vacuum chamber 11 in the form of a right circular cylinder, along with an opening door member 12 for controlling access to the system. A vacuum pump is shown at 13, the pump being coupled to the chamber by the conduit 14.

Also, a vent system for controlling the atmosphere within the chamber is shown generally at 15, and includes a suitable conduit communicating with the chamber, as at 16, along with a suitable control valve 17.

Adjacent the opening to the chamber, an elevator arrangement is shown as at 20, the elevator being arranged to handle a rotary magazine element or the like 21, and raise and lower the individual articles to be coated with selenium, such as the right circular cylindrical members 22-22. A loading fixture is illustrated at 24, this fixture being utilized to transfer the individual articles being coated, such as the articles 22-22, from the magazine member 21 to the unloading fixture 25. The system may accordingly be rendered automatic, or semiautomatic. A closable access hatch is provided in the area of the elevator system 20, to separate effectively or isolate the upper materials handling zone from the zone housing the vacuum chamber.

With attention being re-directed to the chamber 11, it will be seen that a selenium charge retaining crucible is confined within the chamber, such as at 28, this chamber being provided with a substrate access opening such as at 29, this opening being utilized to permit the insertion and extraction of individual articles from the interior of the member 28. As is illustrated in FIGS. 3 and 4, the member 28 is provided with suitable heating elements for the crucible.

Attention is now directed to FIG. 2 of the drawings wherein certain features of the system employing the aspects of the present invention are shown. In this view, a rotating crucible member is shown at 30, with suitable heaters 31 disposed outwardly of the outer surface of the crucible 30. The crucible 30 is arranged to rotate in accordance with the arrow shown at 32. If desired, heat shields may be provided outwardly from the heaters, in order to more carefully control the temperature of the crucible 30 and its neighboring crucibles, if present.

The magazine 34 is provided with a plurality of chambers or the like as at 35, these chambers being disposed radially outwardly of the center of the magazine, and accordingly capable of receiving individual articles to be coated. In the illustration of FIG. 2, the articles being coated are in the form of right circular cylinders which may be hollow sleeve elements. The individual articles to be coated are shown in the chambers as at 36, 37 and 38.

Attention is now directed to the means for inserting and retaining the article to be coated, such as the axially movable collet member generally designated 40. This collet member has an expandable tip portion as at 41, this tip portion 41 having individual temperature sensors disposed adjacent the external surface thereof, with sensor lines in communication with the individual sensors, and shown at 42. Coolant is passed through the individual surfaces of the collet, with coolant fluid being supplied through conduit 43, and passed outwardly through conduit 44. In this fashion, thermal control of the substrate may be accomplished, thereby contributing to uniformity and reproducibility in the finished product.

In the operation of that portion of the system shown in FIG. 2, the expandable collet 41 is inserted into the core of one of the drums retained within the magazine, such as the drum 38, and upon continued forward axial motion of the collet 41, the hollow drum 38 is transferred to the confines or interior of rotating crucible 30 where the deposition of the selenium occurs.

Attention is now directed to FIG. 3 of the drawings wherein the crucible 30 is shown as being retained within a suitable crucible oven. The crucible 30 is fabricated from a suitable refractory material, or metallic structure with a wall thickness capable of withstanding the centrifugal forces encountered, the oven being fabricated from a suitable refractory material or the like. Heaters such as the heating elements 31 are disposed radially outwardly from the outer surface of the rotating crucible 30, these heaters being either radiantly or inductively coupled to the crucible 30 and its contents, and preferably being arranged in equal arcuately spaced relationship about the crucible. The support collet is shown retaining

the hollow drum or sleeve being coated, the article being coated being shown here at 51. The features of the thermally controlling expandable collet are shown in greater detail in FIGS. 4 and 5, and will be discussed hereinafter. For example, one form of temperature sensor is shown at 52, this being a thermocouple which has its hot junction disposed immediately adjacent the surface of the expandable collet. As is apparent from FIG. 5, the expandable collet utilizes a plurality of individual arcuate segments which can be expanded outwardly to make physical contact with the inner surface 53 of drum 51, this contact being a good thermally conductive contact in addition to a mechanical contact. Coolant is provided in and along the bores 55 and 56, with coolant being transmitted through these lines at a rate sufficient to maintain the drum being coated at a temperature of between about 50° C. to 70° C. With coolant moving rapidly through these lines, it is possible to monitor the temperature at the surface of the article 51, without having to experience local warm and local cold areas. The liquid coolant moves in the direction of the arrows shown at 57 and 58.

In order to provide for expansion and contraction of the collet, the interior of the individual segments forming the collet, such as is shown at 60 is in the form of a cone converging toward the right. The expander utilized in combination with this cone is in the form of a conical ramp shaft 61 which is capable of motion in either of two axial directions, so that upon moving to the right, the collet effectively expands and clamps the individual collet segments against the inner surface of the article to be coated. Motion in the opposite axial direction provides for contraction of the individual collet segments. It will be appreciated, of course, that this expansion and contraction arrangement is typical of only one of a variety of such arrangements which could be used in connection with the operation of the present invention.

Attention is now directed to FIG. 4 of the drawings wherein the rotating selenium retaining crucible 30 is illustrated, along with the article to be coated 51. Shutter blades are provided as at 66, these blades being formed with a lenticular profile such as is illustrated in FIG. 5, for the purpose of enhancing the uniformity of the thickness of the selenium coating. These individual shutter blades or baffles have a selenium source viewing surface 70 which is normally hot, and a relatively cooler substrate viewing surface 71. The configuration of the blades shown in FIG. 5 is discussed in greater detail in connection with FIGS. 7A and 7B hereinafter.

It is also possible to heat and/or cool individual shutter blades such as the blades 66, and by the use of such heating or cooling (for example, thermo-electric Joule heat or Peltier cooling) the radial temperature profile can be established for the selenium evaporant and for the substrate. Also, the hot side of the individual blades or baffles can be heated so as to remain free of deposited selenium, while the cold side will, by virtue of its disposition in the arrangement, remain clean since it receives only a small amount of selenium evaporant which is transmitted or returned from the surface of the cooled substrate.

The lenticular configuration for the cross-section of the individual shutter blades is provided in order to permit an effective "throttling" of the deposition rate, thereby permitting a higher temperature in the selenium evaporant, for a given deposition rate. The availability of these shutter elements, therefore, adds certain degrees of freedom for the operator to employ during his coating operation. The lenticular configuration provides for a leveling of the flow of evaporant from the source onto the substrate surface.

Attention is now directed to FIG. 6 of the drawings wherein the axial profile of the individual blades 66 is shown. The reason for the configuration is shown in FIGS. 7A and 7B, wherein the effective source area provides a deposition rate or thickness in the traditional fashion. The end walls of the crucible act as baffles or barrier surfaces, and with the use of blades of the profile shown in FIG. 6, the effective source area is controlled, along with the deposition rate so as to provide a

uniform film thickness along the axial extent of the article being coated.

Better results are also obtained since radiant heat is retained by the crucible in a more uniform fashion. Also, the rate of heat transfer to the substrate is decreased by a factor proportional to the arcuate width of the individual baffles or blades. For a given rate of deposition on a substrate, the total heat transfer to the substrate is actually decreased, this being due to the fact that the rate of evaporation is an exponential function of the temperature, while the radiant gain is the fourth power dependence of radiation upon temperature. Also, as is illustrated in FIG. 8, the individual shutter blades or baffles can be shaped in the axial direction to correct the deposition rate for variations near the end walls, or to accommodate the insertion and withdrawal operations and the consequent time variable incurred for the substrate surface.

It is also recognized that with baffles or blades being employed, the evaporation rate can be controlled with a higher source temperature, thereby enhancing the uniformity of the selenium coating without risking the dangers of uncontrollable substrate temperatures.

During the evaporative deposition, the pressure range of the system will be controlled so that the distance between the surface of the substrate and the surface of the selenium evaporant is less than the mean free path of the selenium in the system. This will assure retention of Knudsen flow, which will eliminate molecular interactions in the flow space. Normally, during evaporative depositions conducted at a source temperature leading to a vapor pressure of between  $10^{-3}$  and  $10^{-4}$  Torr, a charge surface-to-substrate surface of about one centimeter is desirable and useful.

It is normally preferred that the selenium evaporant cover the entire surface of the rotating crucible, thus providing for continuous uniform coating of the substrate with the selenium.

In a typical coating operation conducted in accordance with the present invention, a 9-inch diameter stainless steel crucible is provided having a wall thickness of 1 inch. A charge of selenium is placed in the crucible in a quantity sufficient to provide a charge thickness of more than 1 millimeter. The crucible is then placed within the evaporative system, at a background pressure of preferably less than  $10^{-4}$  Torr, and the temperature is increased to 250° C., with the crucible being rotated at a rate of 300 r.p.m. This operation disposes the selenium charge about the wall of the crucible so as to define a cylindrical charge. The charge is then heated to a temperature of between 180° C. and 230° C., and preferably at a temperature of between 200° C. and 227° C., while rotation is continued at a rate of 300 r.p.m. It has been found that for the lower temperature levels, 100 r.p.m. is adequate to prevent splattering. The substrate is then introduced into the crucible, the substrate having the configuration of the drum 51 in FIG. 4, the axis of the substrate drum being coincidental with the axis of rotation of the crucible. As has been indicated, a spacing of one centimeter is desired between the inner charge surface and the substrate outer surface. So long as this distance is less than the mean free path under the deposition conditions, Knudsen flow characteristics will prevail.

While the substrate is held within the chamber, a substrate temperature of between 50° C. and 70° C. is maintained, with 60

a temperature of 60° C. being considered optimum. For reprographic purposes, the substrate drum is permitted to remain within the crucible for a period of up to about 30 minutes, during which time a film of amorphous selenium having a thickness of between 40 microns and 80 microns will be prepared. Ideally, a film of about 60 microns is preferred for reprographic purposes.

Attention is now directed to FIG. 9 of the drawings wherein a typical finished drum is illustrated, the drum 80 comprising an aluminum substrate member 81 having a dielectric layer 82 separating the surface of the aluminum from the selenium film 83. Ideally, aluminum oxide is formed on the surface of the drum, this surface being prepared by either air-baking, or anodizing operations.

Selenium films prepared in accordance with the present invention have desirable characteristics for reprographic use. Image spreading is minimized because of the high degree of amorphous characteristics in the film. As such, half-tones may be reproduced with a high degree of fidelity. Also, the charge retention is exceptionally long, and the discharge in light is rapid and uniform. When a highly uniform film of aluminum oxide is provided on an aluminum drum, with the oxide layer being preferably between 40 Angstroms and 80 Angstroms in thickness, a high dielectric barrier will be provided to control the dark discharge rate.

I claim:

1. The method of applying a film of amorphous selenium to a substrate having a cylindrical surface which comprises:
  - a. inserting a charge of selenium into a generally cylindrical crucible having an inner wall extending in spaced relationship to a cylindrical axis;
  - b. treating said selenium to dispose the charge along the inner wall of the crucible so as to define a generally cylindrical charge profile spaced about said axis;
  - c. heating said charge to a temperature of between about 180° C. and 230° C.;
  - d. rotating said crucible about its axis at a rate to retain said selenium about said crucible wall;
  - e. inserting said substrate into said crucible with the outer cylindrical surface thereof being spaced at a predetermined distance from the surface of said generally cylindrical charge profile;
  - f. maintaining the temperature of said substrate at a level of between about 50° C. and 70° C. during deposition; and
  - g. thereafter removing said substrate from said crucible.
2. The method as defined in claim 1 being particularly characterized in that the film application to the substrate is conducted in a chamber wherein the selenium source pressure in said chamber is between  $10^{-3}$  and  $10^{-4}$  Torr.
3. The method as defined in claim 2 being particularly characterized in that said selenium is heated to a temperature of between about 200° C. and 227° C. during deposition.
4. The method as defined in claim 1 being particularly characterized in that said cylindrical crucible is rotated at a rate of between about 100 r.p.m. and 300 r.p.m. during deposition.
5. The method as defined in claim 1 being particularly characterized in that said substrate is maintained at a temperature of about 60° C. during deposition.

\* \* \* \* \*